

## UNITED STATES PATENT OFFICE

1,925,910

PRODUCTION OF HARD METAL ALLOYS,  
ESPECIALLY FOR TOOLS

Paul Schwarzkopf and Isidor Hirschl, Reutte,  
Tyrol, Austria; said Hirschl assignor to said  
Schwarzkopf

No Drawing. Application November 16, 1931,  
Serial No. 575,482, and in Germany May 28,  
1931

4 Claims. (Cl. 75—1)

For the production of particularly efficient, hard tools, use is made of carbides of tungsten or molybdenum, which are prepared by fusing or sintering, and are thereupon pulverized and pressed into definite molds and subsequently highly heated. It has proved particularly advantageous to add auxiliary metals to the carbide, and then to sinter the whole, in order to obtain tool materials that are not only extremely hard, but also tough.

In order to obtain tool elements of great hardness, the invention employs neither tungsten alone nor molybdenum alone, also not tungsten-carbide or molybdenum-carbide alone, as suggested heretofore, but a mixture of one or more carbides formed from one or more elements of the sixth group of the periodical system of the elements, comprising molybdenum, tungsten, chromium and one or more carbides of elements of the fourth group of the periodical system comprising titanium, silicon, zirconium.

Such carbides are not used, however, alone, but in accordance with known principles they are employed with auxiliary metals, principally those of the iron group, such as nickel and cobalt, with some chromium, singly or in suitable mixtures. The auxiliary metals are believed to increase the toughness of the alloy or tool produced without, or practically without, changing the composition or structure of the carbides present, although it might be that a kind of diffusion between the auxiliary metals and the carbides, perhaps only in surface layers, takes place while they are heated at sintering temperature, and some kind of surface solution is formed therefore in the hardened alloy.

A hard metal tool element, according to the invention, contains from about 15% to less than 50% carbide of one or more elements of the sixth group, and between about 75% to 39% carbide of one or more elements of the fourth group, the remainder being substantially auxiliary metal of the iron group, with or without chromium, the auxiliary metal amounting altogether to from about 3% to about 22%.

It has been found that surprisingly good results (for example, for high speed material) are obtainable by using 30 to 15% molybdenum-carbide ( $Mo_2C$ ), of the sixth group, and 65 to 70% titanium-carbide ( $TiC$ , with a content of about 20% carbon), of the fourth group, adding hereto as auxiliary metals about 8 to 15% nickel and 0 to 7% chromium. Within this range the optimum seems to be at about 8 to 10% nickel and up to 1 to 2% chromium.

For special other purposes (for example, slower speed material), a mixture of titanium-carbide and molybdenum-carbide in about equal proportions, with auxiliary metal comprising nickel up to 9 and 15% and chromium up to 1 and 2%, has been proved.

Another mixture suitable for the purpose of the invention has been obtained by substituting the titanium-carbide by zirconium-carbide without, however, materially changing the proportions of the constituents.

Surprising results have been further sometimes achieved by adding oxides of metals or metalloids not being reduceable by hydrogen and not, or only at high temperatures, forming carbides. Such oxides are, for example, alumina, silica, the alkaline earths, the group comprising zirconia, and the group comprising the rare earth oxides. Particularly, the addition of alumina in the finest divided form and in relatively small amounts, say up to about 0.5%, has enabled the formation of most suitable alloys of the here-mentioned various compositions.

Comparing a known alloy of tungsten-carbide with about 10% cobalt as auxiliary metal and an alloy of the present invention comprising molybdenum-carbide and titanium-carbide with nickel and chromium as auxiliary metals, the last-mentioned alloy containing, for example, 62% titanium-carbide, 27% molybdenum-carbide, 10% nickel, and 1% chromium, the hardness and toughness will surpass exceedingly that of tungsten-carbide with cobalt. It has been further found that by substituting in the last-mentioned alloy nickel and chromium by cobalt, still better results are achievable than with the alloy containing tungsten-carbide and cobalt.

Any suitable method may in itself be used for the production of the carbides and of the final alloy.

For producing molybdenum-carbide, the following way has proved most convenient. Metallic molybdenum and carbon are mixed in the proportion corresponding to the theoretical values needed for producing the combination  $Mo_2C$ . This mixture is powdered and then heated in a reducing atmosphere up to about 1400 to 1600° C. Hereby the combination is produced containing about 5.9% C., the rest being  $Mo_2$ .

Titanium-carbide can be formed in a similar way from metallic titanium and carbon, the temperatures used being, however, higher, as well understood.

In similar ways, zirconium-carbide and silicon-carbide, etc., can be produced.

Instead of using solid carbon, also gaseous carbon can be used, for example, in the form of carbon or carbon compounds containing gases as coal gas, etc. Such gases are passed over the finely divided metal powders or metal compounds in carbon tubes at temperatures similar to those mentioned before.

The carbides so produced are then powdered again (if necessary) and intimately mixed with the chosen auxiliary metal or metals. Suitable proportions have already been mentioned. The mixtures are then preformed by pressing in suitable molds to a shape similar to the desired shape. Due allowance is, of course, made for the shrinkage which takes place during the following treatment.

The preforming in the molds may be done also under elevated pressure.

The body so preformed and advantageously still under pressure is now to be treated to give it the dense and homogeneous internal structure requisite to its service as a hard metal tool element. This is effected electrically by heavy current led through the body or through the mold.

Any other kind of heating may be employed. The temperature of the body is to be elevated to about 1400 to 1600° C., and this heat treatment is to be continued about one or more hours, or until the desired structure of the body is obtained.

Another way consists in admixing with the powders ready for preforming glycerine, glycol or other alcohols, pressing such mixture, converting the reagents at normal or elevated temperature, driving out totally the unconverted alcohol at about 120 to 200° C., then working and finishing this body of sufficient cohesion, whereupon the sintering is done.

The finished bodies or tool elements may be assembled with other parts to form the tool, or they may themselves directly constitute the tool.

If aluminium-oxide, or similar oxides, as mentioned before, are used as additions in small quantities, then the crystals of heavy metal carbide contained in the body are not materially changed or increased in size by the heat treatment. The crystals are uniformly divided throughout the body. While, otherwise, some diffusion or solid

solution takes place within several carbides and admixed auxiliary metals, such alloying seems to be largely or entirely prevented by addition of the mentioned oxides. This helps to increase or to maintain the toughness of the mass.

It may be mentioned that in cases where oxygen is given off during the heat treatment, such oxides may be obtained by adding to the initial mixture the desired small amounts of the respective metals such as aluminum, silicon, etc., and having them combine with the oxygen freed during the heat treatment.

What we claim is:

1. A hard metal tool element comprising carbide of metal selected from the group consisting of chromium, tungsten and molybdenum and representing from about over 15% up to less than about 50% of the body, and carbide of metal selected from the group consisting of titanium and zirconium, forming between about 39% and about 75% of the body, and the remainder auxiliary metal selected substantially from the iron group of the periodic system.

2. A hard metal tool element comprising carbide of metal selected from the group consisting of titanium and zirconium and carbide of a metal selected from the group consisting of chromium, molybdenum, and tungsten, the content of carbide of the first named group being from about 39% up to about 75%, the content of carbide of the second named group being from about 15% up to about less than 50%, the remainder about 5% to 22% substantially of auxiliary metal of the iron group.

3. A hard metal tool element, containing substantially titanium carbide from about 39% to less than 75% molybdenum-carbide between about 15% and less than 50% and the remainder nickel.

4. A hard metal tool element containing from about 60% to about 75% titanium carbide, about 20% molybdenum carbide, and the remainder substantially from about 5% to about 20% of auxiliary metal taken from the group consisting of cobalt, iron and nickel.

PAUL SCHWARZKOPF.  
ISIDOR HIRSCHL.